

1

3,352,678  
DIFFUSION TRANSFER PHOTOGRAPHIC  
MATERIALS

Fumihiro Nishio, Odawara-shi, Kanagawa-ken, and  
Reiichi Oi and Tatsuya Tajima, Ashigarakami-gun,  
Kanagawa-ken, Japan, assignors to Fuji Shashin  
Film Kabushiki Kaisha, Kanagawa-ken, Japan, a  
corporation of Japan  
No Drawing, Filed Sept. 24, 1963, Ser. No. 311,232  
Claims priority, application Japan, Oct. 5, 1962,  
37/43,019

14 Claims, (Cl. 96—76)

The present invention relates to diffusion transfer photographic materials such as a photographic light sensitive element, a photographic image receiving element, and a developer for diffusion transfer photography, which materials contain a novel toner.

A diffusion transfer photographic process means in general a process comprising exposing a light sensitive element having a light sensitive layer of silver halide to an object or an original image, in the presence of a developer, contacting said light sensitive element with an image receiving element having an image receiving layer containing reducing nuclei such as colloidal silver or silver sulfide capable of reducing silver complex on the surface, whereby the silver halide at the exposed portion of the photosensitive layer is developed and the silver halide at the unexposed portion is dissolved and diffused, followed by depositing on the image-receiving layer as reduced silver, and separating it to obtain a printing image with the object on the image receiving element.

In the case where a toner having an effect on the deposition of reduced silver on the image receiving layer is not used in the present photographic process, the resulting image on the image-receiving layer is not black, but yellow or brown.

The present invention relates to a process for forming a black image on the image-receiving layer by employing a novel toner which has not been described in the prior literatures. According to the present invention, a compound represented by one of the following general formulas is added as a toner into a silver halide emulsion layer, an image-receiving layer, or a developer, or a combination of the said two or three materials,



or



wherein R is a member selected from the group consisting of a lower alkyl group, hydrogen and halogen; Y is a member selected from the group consisting of



2

wherein R<sub>1</sub> and R<sub>2</sub> each represents lower alkyl, aryl, aralkyl, an SO<sub>3</sub>M-substituted alkyl, an —SO<sub>3</sub>M-substituted aryl, an SO<sub>3</sub>M-substituted aralkyl, a COOM-substituted alkyl, a COOM-substituted aryl, a COOM-substituted aralkyl, where M represents H, Na, K or NH<sub>4</sub>, an amino substituted alkyl, an amino substituted aryl, and an amino substituted aralkyl; R<sub>1</sub> and R<sub>2</sub> together may form a divalent alkylene radical and together with an adjacent nitrogen atom may form a heterocyclic ring; and n is a positive integer less than 10.

Examples represented by the above-mentioned general formula are as follows:

COMPOUND 1



COMPOUND 2



COMPOUND 3



COMPOUND 4



COMPOUND 5



COMPOUND 6



COMPOUND 7



COMPOUND 8



3  
COMPOUND 9

## COMPOUND 10



## COMPOUND 11



A mixture of two or more toners may, of course, be used in the method of the present invention.

It is profitable to add these compounds in an amount of 0.001-1 g. per liter of a developer, 0.001-1 g. per kilogram of a silver halide emulsion, and 0.001-1 g. per liter of a solution for forming an image receiving element having an image-receiving layer, respectively. A binder of the silver halide emulsion layer, and the image-receiving layer may be gelatin or the like, or a mixture thereof.

## Example 1

A extra-hard silver chloride emulsion was coated on a photographic paper to form a light sensitive element having the following composition:

|                 | G./m. <sup>2</sup> |
|-----------------|--------------------|
| Silver chloride | 1.2                |
| Benzotriazole   | 0.005              |
| Hydroquinone    | 0.2                |
| Gelatin         | 4.2                |

An original image to be copied was exposed on the dried emulsion layer and treated with a developer having the following composition:

|                                  |     |      |
|----------------------------------|-----|------|
| Hydroquinone                     | g-- | 12   |
| Pyrazone 1-phenyl-3-pyrazolidone | g-- | 0.5  |
| Sodium sulfite (anhydrous)       | g-- | 70   |
| Caustic soda                     | g-- | 15   |
| water to make                    | ml  | 1000 |

During or after development the emulsion layer of the light sensitive element containing the developer was closely in contact with the image-receiving layer of the image receiving element for about 20 seconds. The image receiving element was a coated material on a paper support having the following composition:

|                                | G./m. <sup>2</sup> |
|--------------------------------|--------------------|
| Gelatin                        | 5                  |
| Sodium thiosulfate (anhydrous) | 1.5                |
| Starch                         | 0.5                |
| Colloidal silver sulfide       | 0.002              |
| Compound 1                     | 0.05               |

## 4

By separating the image receiving emulsion layer from the light sensitive emulsion layer, a black positive image was obtained on the image receiving material.

## Example 2

5 Benzotriazole in the light sensitive element employed in Example 1 was replaced with Compound 3 (0.01 g./m.<sup>2</sup>). In this case, even if Compound 1 in the image receiving element was removed, a black positive image 10 was obtained by the same treatment as in Example 1, and stability of the light sensitive emulsion layer was, also, improved.

## Example 3

An original image was exposed by reflection on the 15 same light sensitive element as employed in Example 1, and treated with a developer having the following composition:

|                                  |     |      |
|----------------------------------|-----|------|
| Hydroquinone                     | g-- | 18   |
| Pyrazone 1-phenyl-3-pyrazolidone | g-- | 0.5  |
| Compound 5                       | g-- | 0.05 |
| Sodium sulfite (anhydrous)       | g-- | 60   |
| Sodium thiosulfate (anhydrous)   | g-- | 8    |
| Sodium hydroxide                 | g-- | 14   |
| 25 Water to make                 | ml  | 1000 |

30 By the same treatment as employed in Example 1, the light sensitive emulsion layer containing the developer was closely in contact with the image-receiving layer of the image receiving material having the following composition. In this case, as a support for the image receiving material, paper or transparent base could be used.

|                           | G./m. <sup>2</sup> |
|---------------------------|--------------------|
| Gelatin                   | 4                  |
| 35 Polyvinyl alcohol      | 1.5                |
| Compound 7                | 0.06               |
| Barium sulfate            | 0.4                |
| Palladium sulfide colloid | 0.003              |

40 When the image-receiving layer of the image receiving material was separated from the light sensitive emulsion layer a black image was obtained on the image-receiving layer of the image receiving material. In this case, scum on the surface of the image receiving image could be removed.

## Example 4

45 Compound 5 in the developer in Example 3 was replaced with Compound 2 (0.02 g./1000 ml.) and Compound 7 in the image-receiving layer of the image receiving element was replaced with Compound 8 (0.05 g./m.<sup>2</sup>) in Example 3. The same treatment as in Example 3 was carried out to obtain a black positive image.

What we claim is:

50 1. In a diffusion transfer photographic composition containing a first member selected from the group consisting of a light sensitive silver halide composition, an image receiving composition, and a developer; the improvement comprising at least one toner having a formula selected from the group consisting of



70 wherein R represents a member selected from the group consisting of a lower alkyl group, hydrogen, and a halogen.

atom; Y represents a member selected from the group consisting of



wherein  $R_1$  and  $R_2$  each represents lower alkyl, aryl, aralkyl, a  $-SO_3M$ -substituted alkyl, a  $SO_3M$ -substituted aryl, a  $SO_3M$ -substituted aralkyl, a  $COOM$ -substituted alkyl, a  $COOM$ -substituted aryl, a  $COOM$ -substituted aralkyl, where M represents H, Na, K, or  $NH_4$ , an amino substituted alkyl, an amino substituted aryl, and an amino substituted aralkyl; and wherein  $R_1$  and  $R_2$  together may form a divalent alkylene radical and  $R_1$  and  $R_2$  together with an adjacent nitrogen atom may form a heterocyclic ring; and  $n$  is a positive integer less than 10.

2. A composition according to claim 1, wherein said first member is a light sensitive silver halide composition.

3. A composition according to claim 1, wherein said first member is an image receiving composition.

4. A composition according to claim 1, wherein said first member is a developer.

5. A composition according to claim 1, wherein  $R_1$  and  $R_2$  together with an adjacent nitrogen atom form a heterocyclic ring.

6. A composition according to claim 5, wherein said heterocyclic ring contains a member selected from the group consisting of oxygen and sulphur.

7. A composition according to claim 6, wherein the toner has the formula (A).

8. A composition according to claim 1, wherein the toner has the formula (B), and Y is



9. A composition according to claim 1, wherein the toner is



10. A composition according to claim 1, wherein the toner is



11. A composition according to claim 1, wherein the toner is



12. A composition according to claim 1, wherein the toner is



13. A composition according to claim 1, wherein the toner is



14. A composition according to claim 1, wherein the toner is



No references cited.

45 J. TRAVIS BROWN, *Acting Primary Examiner.*

NORMAN G. TORCHIN, *Examiner.*

C. E. DAVIS, *Assistant Examiner.*